

# United States Patent Office

3,132,101

Patented May 5, 1964

1

3,132,101

DETERGENT AND ANTI-OXIDANT LUBRICANT  
Manley Kjonaas, Hammond, Ind., assignor, by mesne  
assignments, to Sinclair Research, Inc., New York,  
N.Y., a corporation of Delaware  
No Drawing. Filed May 21, 1956, Ser. No. 585,979  
4 Claims. (Cl. 252—32.7)

The present invention relates to a mineral oil composition and more particularly to the use of a novel additive to impart antioxidant and detergent properties to lubricating oils.

Various detergent additives have heretofore been proposed for use in mineral oil compositions, such as heavy duty lubricating oils, which are suitable for use as crankcase lubricants for internal combustion engines, including automobile, diesel and marine engines, which operate for long periods of time at high temperatures and in which the lubricant comes in contact with metal surfaces. In general, the function of these detergent additives, such as, for example, the alkaline-earth metal salts of petroleum sulfonic acids, is to impart properties to the motor oil which will enable it to keep the pistons, rings and valves free of varnish and lacquer deposits by keeping oil oxidation products and other types of insoluble matter in suspension or dispersion so that these materials will not settle out and adhere to metal surfaces. The oil-soluble metal salts of the petroleum sulfonic acids are among the most widely used additive agents to improve the detergent properties of lubricating oils. However, while these detergent additives perform satisfactorily in dispersing sludge and preventing lacquer deposits, many of these additives, particularly under extreme operating conditions, increase the rate of oxidation of the oil and their presence effects an increase in the concentration of acidic oxidation products and thus an increased rate of corrosion to the bearings, pistons, valves and the like.

In accordance with my invention, I have discovered a new and useful detergent-antioxidant additive prepared by reacting basic barium petroleum sulfonate with a phosphorus sulfide-hydrocarbon reaction product. I have found that this combination of constituents produces a detergent material having particularly desirable properties for use in lubricating oils, including sludge dispersant properties, anti-wear properties and the prevention of varnish formation and lacquer-like deposits. The useful additives of my invention provide lubricating oil compositions with improved resistance to oxidative deterioration whereby corrosion to valves, bearings, pistons and the like, is reduced rather than accelerated.

The novel detergent-antioxidant lubricating oil additives of this invention can be employed in amounts varying over a considerable range depending upon the intended purpose of the resultant composition and the conditions under which it is to be used. In compositions intended for use as crankcase lubricants for internal combustion engines, the proportion of additive based on the total weight of the mineral oil composition, may range from 0.01 to 20.0 weight percent, preferably is from about 0.5 to 10.0 weight percent. In addition, the lubricant composition advantageously may contain from about 0.001 to 5 weight percent of anti-wear agents and anti-oxidants such as elemental sulfur, zinc dithiophosphate, or other organic sulfur compounds, such as sul-

2

furized sperm oil and the like. Furthermore, the lubricant may contain other agents such as dyes, pour depressors, thickeners, viscosity index improvers and any of agents conventionally used as additives for lubricating oils.

In carrying out the preparation of the additives of this invention it is preferred to use chemically equivalent quantities of the reactants so as to obtain a neutral product. However, if a basic oil blend is desired than less than the chemical equivalent amount of the phosphorus sulfide-hydrocarbon material should be used, preferably not less than about 50 percent of the equivalent amount, to obtain the reaction product and unreacted basic barium sulfonate.

15 The reaction between the basic barium sulfonate and the phosphorus sulfide-hydrocarbon material is carried out by mixing the materials at a temperature of from about room temperature to 500° F. or more, preferably about 150 to 200° F. until the reaction is complete. Ordinarily, 20 after about one hour the reaction is considered complete, although at lower temperatures, e.g. 160 to 180° F., the product is thereafter heated to about 250 to 300° F. to remove the water of reaction. Although my new additive is described as a reaction product, I do not wish to 25 be bound by this theory as there may in fact not be a reaction effected.

The basic organic sulfonates employed in the preparation of the lubricating compositions of my invention are the barium salts derived from the oil-soluble sulfonic acids produced in the treatment of petroleum hydrocarbons with a sulfonating agent such as sulfuric acid or sulfur trioxide. The preferentially oil-soluble sulfonic acids, generally referred to as mahogany acids, are conveniently employed as a concentrate in the oil from which 30 they are derived and may be prepared by sulfonating a suitable petroleum distillate with fuming sulfuric acid to obtain approximately a 10 weight percent concentration of mahogany acid in the acid oil, or by sulfonating with sulfur trioxide, in which case approximately a 20 weight 35 percent concentration is obtained. The useful mahogany acids, which generally have a molecular weight of about 300 to 500 or higher, normally show a titratable acidity and may be converted into the basic barium salts by 40 neutralization of the acid oil with an excess of basic metal compound to obtain a basic barium sulfonate of higher metal content than the normal salt. In the preparation of the basic petroleum sulfonates, the amount of barium metal in excess of that theoretically required to replace 45 the acidic hydrogens of the sulfonic acids should be at least 1.5 equivalents as determined from the acid number of the acid oil. Advantageously, if desired, the basic metal sulfonate can be carbonated by treatment with carbon dioxide at atmospheric or slightly elevated pressure until the strong basicity of the sulfonate is reduced from 50 a pH of about 14 to a pH between about 7 to 8. In the practice of this invention the basic barium sulfonate is prepared by neutralizing a sulfonated sweet West Texas gas oil fraction with a theoretical excess of barium oxide. Although the mahogany acids contain a sulfonate concentration of about 10%, introduction of barium (3.5%) 55 gives a barium sulfonate concentration of about 13%.

The phosphorus sulfide-hydrocarbon materials which are employed in the present invention to produce the novel lubricating oil additives are the reaction products of a

sulfide of phosphorus with a suitable hydrocarbon material of lubricating viscosity such as a material of natural petroleum origin, for example, a heavy hydrocarbon oil of lubricating viscosity having a molecular weight above 500, i.e., residual lubricating oils, or a synthetic hydrocarbon material such as an olefin or olefin polymer having a molecular weight of from about 400 to 2000 or more. The sulfide of phosphorus which may be employed with the hydrocarbon material is preferably phosphorus pentasulfide,  $P_2S_5$ , although  $P_3S_3$ ,  $P_4S_7$  or other phosphorus sulfides or mixtures thereof can be used. Ordinarily, the phosphorus sulfide-hydrocarbon reaction is carried out at a temperature of from about 200 to 500° F., preferably about 400 to 500° F., and in a non-oxidizing atmosphere, such as an atmosphere of nitrogen. The amount of phosphorus sulfide which can be used may range from 1 percent to 50 weight percent and is preferably from about 5 percent to 25 percent of the hydrocarbon material. The final reaction product will usually contain from about 1 to 6% by weight of organically combined phosphorus.

In a preferred embodiment, a hydrocarbon material such as a mineral oil bright stock or cylinder stock having a viscosity within a range of about 120 to 300 SUS at 210° F. is reacted with 7 to 17 weight percent of phosphorus penta-sulfide at a temperature between about 400 to 500° F. for a period of about 10 to 20 hours. By reacting a phosphorus sulfide with a bright stock for example, the formation of oil-insoluble products which are pro-sludging in typical lubricating oil blends are greatly reduced as compared to the reaction with a lighter oil, such as a neutral oil, which affords a larger percentage of insoluble reaction products. Ordinarily, if the reaction mixture contains insoluble products these materials can be removed by filtration or centrifugation performed at an elevated temperature, usually about 150 to 280° F. Other suitable hydrocarbon oils which can be reacted with phosphorus sulfide include olefins such as cetene, melene, high molecular weight alkenes obtained by cracking petroleum oils, etc. and olefin polymers such as those obtained from the liquid phase polymerization of butylene and isobutylene in the presence of a Friedel-Crafts type catalyst.

The base mineral oil used in the preparation of the lubricating composition will ordinarily depend upon the purpose for which the composition is intended and its service application. When the compounded oil is to be used for the lubrication and protection of internal combustion engines, it is preferred to use a blend of conventionally finished Mid-Continent neutrals and Mid-Continent bright stocks. Other lubricating oil fractions or blends may be used to meet special lubricating requirements.

The method of preparing the additives of the present invention and their use in lubricating oils are illustrated in the following examples. These examples are given for illustrative purposes only and are not to be considered as limiting the scope of the invention.

The following example illustrates the preparation of basic barium sulfonate.

#### EXAMPLE I

A sweet West Texas gas oil fraction having a viscosity of 270 SUS at 100° F. was treated with four 28 pounds per barrel dumps of 20% oleum. After each dump of oleum the sludge was removed. After all of the oleum was added the acid-treated oil was blown with air to remove  $SO_2$ . The acid-treated oil contained approximately 10% mahogany sulfonic acid and had an acid number of 14.1. Thereafter the acid oil was neutralized with approximately 250% theoretical barium oxide in a water

solution for several hours at 160 to 180° F. followed by dehydration by raising the temperature to 300° F. The product was filtered with Super-Cel to leave a basic barium sulfonate which analyzed as follows:

5 Percent barium ..... 13.36  
Base number to pH 4 ..... 13.9

<sup>1</sup> The percent barium for the normal salt is 1.7.

10 The method of preparing the phosphorus sulfide-hydrocarbon reaction product is described in Examples II and III.

#### EXAMPLE II

15 1106 gallons of a Mid-Continent bright stock having a viscosity of 120 SUS at 210° F. were charged to the reaction kettle and heated to 275° F. 1200 pounds of  $P_2S_5$  were added while stirring the mixture and the temperature was maintained at 440° F. for 14 hours. The reaction mixture was cooled to 275° F. and filtered with Super-Cel to leave a product which analyzed as follows:

Percent sulfur ..... 5.78  
Percent phosphorus ..... 3.13  
25 Acid number ..... 32.7

#### EXAMPLE III

30 8500 pounds of Pennsylvania bright stock, viscosity 150 SUS at 210° F., were charged to the reaction kettle and heated to 275° F. 1500 pounds of  $P_2S_5$  were added with stirring and the temperature was maintained at 440° F. for 14 hours. The reaction mixture was cooled to 275° F. and filtered with Super-Cel to give a product

35 which analyzed as follows:

Percent sulfur ..... 7.36  
Percent phosphorus ..... 4.11  
40 Acid number ..... 42.3

40 The following examples illustrate the method of preparing my new additive by reacting basic barium sulfonate with a phosphorus sulfide-hydrocarbon reaction product.

45 In Example VI the amount of  $P_2S_5$ -hydrocarbon reaction product employed was that calculated to neutralize the basic barium sulfonate. The product thus obtained is substantially neutral. Example V was prepared by using less than the equivalent amount of  $P_2S_5$ -hydrocarbon material so as to obtain a basic product.

#### EXAMPLE IV

55 10,000 grams of basic barium sulfonate concentrate, as prepared in Example I, were mixed with 3,640 grams of  $P_2S_5$ -bright stock reaction product, as prepared in Example II, and heated to a temperature of 160 to 180° F. until the reaction was complete. The reaction mixture was then heated to 300° F. to remove the water of reaction. The product analyzed as follows:

Percent barium ..... 2.46  
Percent phosphorus ..... 0.82  
60 Percent sulfur ..... 1.98  
Base number to pH 4 ..... 0.00

#### EXAMPLE V

70 6810 grams of basic barium sulfonate concentrate, as prepared in Example I but containing 3.58% barium and having a base number to pH 4 of 13.6, were mixed with 563 grams of  $P_2S_5$ -hydrocarbon reaction product as prepared in Example III. The mixture was heated to 160 to 180° F. for one-half hour and then heated to 250° F. to

remove the water of reaction. The product analyzed as follows:

|                     |      |
|---------------------|------|
| Percent barium      | 3.28 |
| Percent phosphorus  | 0.30 |
| Base number to pH 4 | 5.94 |

The effectiveness of the barium-P<sub>2</sub>S<sub>5</sub>-bright stock reaction product in imparting anti-wear properties to lubricating oils is demonstrated by the LS-5 valve train wear test. The LS-5 engine test is run in a 1953 Chevrolet Powerglide engine with 235 cubic inch displacement. The hydraulic valve lifters are made of chilled cast iron, the camshaft of forged steel and the rocker arms of malleable iron. The test duration is 24 hours at an engine speed of 3150 r.p.m. and with a load of 30 brake horsepower. The oil sump temperature is maintained at 255° F. and the valve springs are loaded to 150% of the normal static load. In this test the faces of the 12 hydraulic valve lifters tend to spall or pit if the oil is deficient in this particular type of anti-wear property.

Reaction products of either hydrocarbon-P<sub>2</sub>S<sub>5</sub> or steamed hydrocarbon-P<sub>2</sub>S<sub>5</sub> with basic barium sulfonate were blended to the same barium content (0.9%) as the reference oil. The reference oil used was an SAE 10W oil containing basic barium sulfonate, a zinc dialkyl dithiophosphate, viscosity index improver and foam inhibitor. It analyzed 0.9% barium and 0.09% phosphorus. Except for the replacement of the basic barium sulfonate with the specified new reaction products, the blends were identical with the reference oils. The following table shows the improved anti-wear properties resulting from the use of the new reaction products.

Table I

## LS-5 ENGINE TEST RESULTS

| Additive                                                                  | Additive Concentrate as Prepared in Ex. No.— | Amount of Additive Concentrate, Wt. percent | No. of Spalled Valve Lifters |
|---------------------------------------------------------------------------|----------------------------------------------|---------------------------------------------|------------------------------|
| Basic Barium Sulfonate of Reference Oil                                   | I                                            | 27.7                                        | 11                           |
| Basic Barium Sulfonate-Oil-P <sub>2</sub> S <sub>5</sub> Reaction Product | V                                            | 28.5                                        | 4                            |

Table II illustrates the ability of the new additives to increase the anti-oxidation characteristics of lubricating oils in which they are contained. The oxygen absorption tests were run at 360° F. with a copper-lead catalyst on blends containing the new reaction products at 0.52% barium level in a 95 viscosity index solvent-treated Mid-Continent neutral oil of about 160 viscosity SUS at 100° F. As compared to the conventional basic detergents the new reaction products show increased oxidation resistance. Results of oxygen adsorption tests are listed in the following table.

Table II

|    | Additive                                                                  | Additive Concentrate as Prepared in Ex. No.— | Amount of Additive Concentrate, Wt. percent in Base Oil | Rate of Oxygen Absorption Per 100 g. of Blend |
|----|---------------------------------------------------------------------------|----------------------------------------------|---------------------------------------------------------|-----------------------------------------------|
| 5  | Basic Barium Sulfonate                                                    | I                                            | 15.5                                                    | 2,200 cc. in 56 minutes.                      |
| 10 | Basic Barium Sulfonate-Oil-P <sub>2</sub> S <sub>5</sub> Reaction Product | IV                                           | 21.1                                                    | 1,656 cc. in 300 minutes.                     |

I claim:

1. A lubricating oil composition consisting essentially of a mineral lubricating oil and from 0.01 to 20.0 weight percent of a product obtained by (1) contacting at a temperature of from about room temperature to 500° F. an oil-soluble basic barium petroleum sulfonate with not less than about 50 percent of the equivalent amount of an oil-soluble phosphorus sulfide-mineral oil bright stock reaction product, said bright stock being of lubricating viscosity and having a molecular weight above 500, and (2) removing water from the product, said water resulting from said contacting.
2. The composition of claim 1 wherein said lubricating composition contains 0.5 to 10.0 weight percent of said contacting product.
3. The composition of claim 1 wherein a chemically equivalent quantity of said phosphorus sulfide bright stock reaction product is contacted with said sulfonate so as to obtain a substantially neutral product.
4. The composition of claim 1 wherein said phosphorus sulfide-bright stock product is prepared by reacting 7 to 17 weight percent of phosphorus pentasulfide with a mineral oil bright stock having a viscosity within the range of about 120 to 300 SUS at 210° F. at a temperature between about 400 to 500° F. for a period of about 10 to 20 hours.

40

## References Cited in the file of this patent

## UNITED STATES PATENTS

|           |                 |               |
|-----------|-----------------|---------------|
| 2,419,584 | Noland          | Apr. 29, 1947 |
| 2,421,004 | Berger et al.   | May 27, 1947  |
| 2,476,813 | Buckmann et al. | July 19, 1949 |
| 2,476,972 | Fuller et al.   | July 26, 1949 |
| 2,493,216 | Berger et al.   | Jan. 3, 1950  |
| 2,538,696 | May             | Jan. 16, 1951 |
| 2,546,552 | Loane et al.    | Mar. 27, 1951 |
| 2,623,016 | Mertes          | Dec. 23, 1952 |
| 2,681,891 | Bos et al.      | June 22, 1954 |
| 2,723,236 | Asseff et al.   | Nov. 8, 1955  |
| 2,767,164 | Asseff et al.   | Oct. 16, 1956 |
| 2,798,045 | Buck et al.     | July 2, 1957  |
| 2,969,324 | Knapp et al.    | Jan. 24, 1961 |